

April 2, 1940.

J. R. BALDER

2,195,846

## CUTLERY

Original Filed May 29, 1937



INVENTOR  
JOHN R. BALDER  
BY *John R. Balder*  
ATTORNEY

## UNITED STATES PATENT OFFICE

2,195,846

## CUTLERY

John E. Balder, Stratford, Conn., assignor to Remington Arms Company, Inc., a corporation of Delaware.

Application May 29, 1937, Serial No. 145,546  
Renewed February 20, 1940

## 3 Claims. (CL. 30—164)

This invention relates to the art of and means for retarding rust and corrosion on the bare steel surfaces of a cutting blade and cooperative steel parts in an implement of cutlery, particularly a pocket knife wherein the contiguity of such parts and the unavoidable presence of moisture are highly conducive to such rust and corrosion.

As commonly constructed, the blades and the blade positioning springs of a pocket knife are subject to rubbing engagement with each other, and are further subject to contact and sliding engagement with metallic linings or partitions in the hollow handle of the knife, which linings or partitions are commonly known as "scales" and between which scales the blades of the knife are pocketed or sheathed when folded into closed relation to the handle.

An object of the invention is to reduce the tendency of the cutting blade and its cooperative positioning spring to rust when these parts are made of grades of high carbon steel best capable of supporting a good cutting edge and of possessing good spring action, such steel being preferably unalloyed with any metals detrimental to these qualities. So-called "stainless steel" not only is less satisfactory in these qualities but is more costly. Hence a companion object is to produce a comparatively rust-proof knife which at the same time is more economical to manufacture.

Another object of the invention is to retard rusting or corrosion of bare surfaced steel working parts such as the cutting blade of a folding knife without coating the surface of the blade with any rust preventive material different from that of which its body is composed.

A further object is to retard electrochemical activity that might otherwise be set up by the dwelling of wet substances or moist air between contiguous parts of rust susceptible metal, by interposing between the metallic bodies of the parts a different material or metal possessing a higher natural electric potential than that possessed by the metal or metals comprising the bodies of the parts.

A specific object of the invention is to protect the cutting blade or blades of a pocket knife from rust or corrosion from the above causes by coating the adjacent surfaces of the "scales" of the knife with a material possessing properties peculiarly effective for the purpose, which properties have been discovered to reside in the metals, zinc and cadmium.

These and other objects of the invention will be clearly understood from the following descrip-

tion in which reference is had to the accompanying drawing wherein:

Fig. 1 is an edgewise view of a two-blade pocket knife embodying the present improvements, in which one of the blades is shown in open position and the other blade is closed.

Fig. 2 is a side elevation of the knife with the blades positioned as in Fig. 1.

Fig. 3 is a view of the handle portion of the knife taken in cross section on the longitudinal plane 3—3 in Fig. 1 looking in the direction of the arrows, the open blade being partially broken away.

Fig. 4 is a sectional view taken on the planes 4—4 in Fig. 1 looking in the direction of the arrows and is drawn on a much enlarged scale.

Fig. 5 is a perspective view of one of the scales or partitions of the knife handle structure detached from its associated parts.

Fig. 6 is a sectional view drawn on a scale intermediate that of Fig. 1 and Fig. 4 and is taken on the planes 6—6 in Fig. 3 looking in the direction of the arrows, showing only the scale and the exterior parts of the handle which are riveted thereto.

Fig. 7 is a transverse sectional view through a scale of the knife drawn to much larger proportions than in Fig. 4 to illustrate the metallic coating thereon.

While the principles which underlie these improvements may be availed of in any article of cutlery wherein a steel blade is sheathed or pocketed so as to lie partly in contact with or very close to the metallic lining of an enclosing structure, they are illustrated herein as embodied in the conventional arrangement of the parts of a pocket knife having the large blade 10 and the smaller blade 11.

The handle structure of the knife comprises a central partition scale 12 interposed between the blades from end to end of the handle and two similar composite exterior walls each of whose structure may be as represented in Fig. 6. Each wall structure may comprise a lining scale 13 to each end of which are secured respectively the tips or bolsters 14 and 15 providing a longitudinal recess therebetween which may be filled with a body 16 of bone, horn, or any other material suitable to be grasped by the hand and secured in place by any means commonly employed.

The partition scale 12 and both lining scales 13 are surface coated preferably with zinc for purposes which will hereinafter be more fully explained and in keeping with important objectives

of this invention. This coating is indicated at 24.

A cantilever spring 17, commonly of the shape shown in Fig. 3, is interposed between the partition scale 12 and one of the lining scales 13, and 5 a similarly shaped but narrower spring 18 is similarly positioned between the partition scale 12 and the other lining scale 13. The left end of springs 17 and 18 in Figs. 1, 2 and 3, are rigid with and serve to space the said three scales being secured therebetween by through-rivets 19. 10 A similar rivet 20 extends transversely through the entire handle structure including springs 17 and 18 near the central portion of the latter. The right ends of springs 17 and 18 bear upwardly 15 against the tangs 21 and 22 respectively of blades 16 and 14, being free to slide somewhat between the scales.

A pintle 23 serves as common pivot for both blades in the well known manner which blades 20 are thus adapted to fold between open and closed 20 positions by swinging while in actual contact with, or closely contiguous to, the scales of the handle structure which flank them. Fig. 4 makes plain that portions of the blades remote from 25 their pivoted ends may also contact or lie closely adjacent the handle scales.

It has long been a problem to contend successfully with the strong tendency to rust and corrosion which is aggravated by the juxtaposition of parts illustrated in Fig. 4 when moisture 30 is present, as is bound to be the case from many wet uses to which a pocket knife is put and from its habitual nearness to body moisture when carried on the person.

35 Heretofore corrosion and rusting of liners and scales has been obviated by making these parts of such difficulty corrodible metals as brass and nickel silver. These metals are relatively expensive, and experiments leading to the present invention have shown that in close proximity to the back springs and blades of a pocket knife when carried on the person they actually accelerate rusting of the steel parts.

It has been found that the rusting of steel 40 back springs and especially steel blades in an implement of the type of a pocket knife is minimized and often substantially prevented by the use of scales or liners surfaced with a metal having an electrical potential which is positive with 45 respect to the potential of iron. Outstanding among such metals are cadmium and zinc. An accelerated rusting test, conducted by exposing samples to a salt spray for a period of a few hours, gave substantially no rusting of blades in recesses having zinc-surfaced scales; whereas, 50 scales having surfaces of metals having a potential which is negative with respect to iron showed very destructive rusting.

The knife with the blades closed may be re-

garded as an electrolytic cell, of which the scale and the blades form poles separated by a narrow gap of moist and impure air. Outside of the cell the blade and scale are short-circuited through the blade tang and blade pivot. The 5 flow of the current within the cell is from the zinc scale to the blade; thus, electrolytic action does not tend to attack and remove the material of the blade as it does when the flow of current is away from the blade.

10 Within the present invention, scales may be made wholly of zinc or other metal having an electrical potential higher than that of iron, but preferably they are made from such a relatively inexpensive material as soft iron or mild steel 15 which has been surface coated with the metal of higher potential by any well-known coating process which is effective to provide a continuous and adherent coating. The coating is preferably applied while the metal is in strip or sheet 20 form, and scale blanks of proper configuration are struck from the coated sheet. A substantial improvement in the quality of articles of the type of pocket knives as heretofore described is thus brought about simultaneously with a material reduction in manufacturing cost.

25 In its broader scope the invention is not limited to the method herein proposed by which zinc may be interposed between the steel parts of a knife, nor to any particular manner of coating the surface of the scales of a knife with zinc or corresponding metal, wherefore the appended claims are to be interpreted as inclusive of all means which may come within their terms for seizing upon the principles employed in these 30 improvements.

35 I claim:

1. In an implement of cutlery in combination, a handle structure including a scale, a ferrous metal blade pivotally connected to the handle structure to swing in a plane contiguous to but spaced from said scale, and a coating of zinc 40 covering the surface of said scale facing said blade, whereby corrosion of said blade is substantially inhibited.

2. In a pocket knife including a hollow handle, scales lining the interior of said handle, a steel blade foldable into pocketed and spaced relation to said handle between said scales, and a coating of zinc carried on the surfaces of said scales 45 facing said blade, whereby corrosion of said steel blade is substantially inhibited.

3. A pocket knife comprising a steel back spring, a steel blade, and a scale in spaced relation to said blade having a surface of zinc facing 50 said blade, whereby corrosion of said steel parts is substantially inhibited.

JOHN R. BALDER.